

# United States Patent

[11] 3,615,906

[72] Inventors Marvin C. Vanwanderham;  
John A. Harris, Jr., Palm Beach, Fla.;  
James J. Campbell, Cincinnati, Ohio  
[21] Appl. No. 811,201  
[22] Filed Mar. 27, 1969  
[45] Patented Oct. 26, 1971  
[73] Assignee United Aircraft Corporation  
East Hartford, Conn.

[54] **PROCESS FOR FABRICATING THREADED  
ELEMENTS FROM THE AGE-HARDENABLE  
ALLOYS**

6 Claims, No Drawings

[52] U.S. Cl..... 148/12.7,  
148/12.3  
[51] Int. Cl..... C22f 1/00,  
C22f 1/10, C21d 9/00  
[50] Field of Search..... 148/12.3,  
11.5, 12.7

[56]

**References Cited**

**UNITED STATES PATENTS**

|           |         |                   |          |
|-----------|---------|-------------------|----------|
| 2,637,672 | 5/1953  | Losco et al. .... | 148/12.3 |
| 2,957,790 | 10/1960 | Metcalfe ....     | 148/12.3 |
| 3,357,868 | 12/1967 | Tanczyn ....      | 148/12.3 |
| 3,376,780 | 4/1968  | Tanczyn ....      | 148/12.3 |

*Primary Examiner—L. Dewayne Rutledge*

*Assistant Examiner—W. W. Stallard*

*Attorney—Richard N. James*

**ABSTRACT:** Threaded elements having improved mechanical properties for high-temperature service are fabricated from the age-hardenable superalloys in a process comprising: solution heat treating the alloy and establishing a grain size corresponding to ASTM 2-6, or more preferably ASTM 4-5; forming the threads; stabilization heat treating the threaded alloy; and aging.

**PROCESS FOR FABRICATING THREADED ELEMENTS  
FROM THE AGE-HARDENABLE ALLOYS**

**BACKGROUND OF THE INVENTION**

The present invention relates to the production of threaded elements from the age-hardenable superalloys.

In gas turbine engines, a number of threaded elements, such as bolts and compressor tie rods, are utilized in environments involving exposure under stress to elevated temperatures. As manufactured by conventional techniques, these elements are prone to failure with time, due primarily to poor stress relaxation resistance and insufficient thread strength.

Two alloys, Waspaloy and Astroloy, are widely used in applications of this nature, although other age-hardenable alloys such as Inco 901, Inconel x 750 and Udiment 700, are also available for this type of service. Waspaloy, which is suitable for this type of service up to temperatures of about 1,200° F., has the following nominal composition by weight: 19.5% Cr, 13.5% Co, 0.07% C, 3% Ti, 1.4% Al, 4% Mo, 0.005% B, 0.08% Zr, bal. Ni. For service over 1,200° F., Astroloy is commonly used at a nominal composition, by weight of: 15.5% Cr, 17% Co, 0.07% C, 3.3% Ti, 4.5% Al, 5.3% Mo, 0.03% B, bal. Ni.

The conventional threading practice involves rolling of the threads in barstock after the stabilization heat treatment but prior to aging. Threaded elements so formed, however, exhibit poor stress relaxation and thread failure resistance and, hence, are prone to thread failure in service.

**SUMMARY OF THE INVENTION**

The present invention describes a fabrication technique for providing threaded elements from the age-hardenable alloys characterized by improved mechanical properties in elevated temperature applications.

The improved properties are achieved by first establishing a grain size of ASTM 2-6 by appropriate heat treatment and, then, by altering the conventional thread forming procedure to provide rolling of the threads prior to stabilization and aging. The process thus involves:

solution heat treating the alloy to establish a grain size of ASTM 2-6 or more preferably ASTM 4-5;

forming the threads;

stabilizing heat treating the threaded alloy; and aging.

**DESCRIPTION OF THE PREFERRED EMBODIMENTS**

For service to temperatures up to about 1,200° F., suitable stock is formed from an alloy consisting of, by weight: 18-21 percent chromium, 12-15 percent cobalt, 0.04-0.10 percent carbon, 3.5-5 percent molybdenum, 2.75-3.25 percent titanium, 1.2-1.6 percent aluminum, 0.02-0.08 percent zirconium, 0.003-0.01 percent boron, balance essentially nickel. The stock is solution heat treated at a temperature of about 1,825°-1,900° F. for 2-4 hours and cooled at a rate equivalent to air cool or faster the conditions being selected to establish a grain size of ASTM 2-6, preferably ASTM 4-5. Any machining of boltheads, etc., may be done either before or after the solution heat treatment. Threads are formed by a single rolling process. After thread rolling, the parts are stabilization heat treated by heating to about 1,550° F.; holding at heat for about 4 hours; and cooling in air. After stabilization, the parts are precipitation heat treated by heating to about 1,400° F.; holding at heat for about 16 hours; and cooling in air.

For service in excess of about 1,200° F., the stock is formed from a preferred composition consisting of, by weight: 14-16 percent chromium, 16-18 percent cobalt, 0.03-0.09 percent carbon, 4.5-5.5 percent molybdenum, 3.35-3.65 percent titanium, 3.85-4.15 percent aluminum, 0.02-0.03 percent boron, balance essentially nickel. The stock is solution heat treated at a temperature of 1,975° F. or higher, held at temperature to establish a grain size corresponding to ASTM 2-6, preferably 4-5; and cooled at a rate equivalent to air cool or faster. Threads are formed in a single rolling process. After thread rolling, parts are stabilizing heat treated by: holding the

part at a temperature of about 1,600° F., for about 8 hours; and cooling at a rate equivalent to air cooling. The parts are subsequently precipitation heat treated at about 1,200° F. for 24 hours and air cooled; and heat treated at about 1,400° F. for about 8 hours and air cooled.

A number of specimens were prepared with varying heat treatments as affecting grain size and were subjected to a variety of tests comparing the effect of both grain size and the processing sequence. The results of a number of these tests are summarized in the following tables.

TABLE I

Specimen Grain Size/Threading Practice

| Part No. | Predominant Grain Size ASTM | Combinations Threading Practice          |
|----------|-----------------------------|------------------------------------------|
| 9561     | 0-2                         | Roll threads, solution, stabilize, age.  |
| 9562     | 0-2                         | Solution, roll threads, stabilize, age.  |
| 9563     | 0-2                         | Solution, stabilize, roll threads, age.  |
| 9564     | 0-2                         | Solution, stabilize, age, roll threads.  |
| 9565     | 0-2                         | Solution, stabilize, age, grind threads. |
| 9571     | 5-7                         | Roll threads, solution, stabilize age.   |
| 9572     | 5-7                         | Solution, roll threads, stabilize, age.  |
| 9573     | 5-7                         | Solution, stabilize, roll threads, age.  |
| 9574     | 5-7                         | Solution, stabilize, age, roll threads.  |
| 9575     | 5-7                         | Solution, stabilize, age, grind threads. |

TABLE II

Room Temperature Tensile Results and Specimen Data

| CKB | Grain Size Number | YS, K s.i. | UTS, K s.i. | EL, % | RA, % | Failure Location |
|-----|-------------------|------------|-------------|-------|-------|------------------|
| 40  | 9561              | 133        | 210         | 21    | 16    | Threads          |
|     |                   | 130        | 208         | 21    | 19    | Shank            |
|     |                   | 123        | 180         | 15    | 13    | Shank            |
| 45  | 9562              | 125        | 192         | 18    | 16    | Shank            |
|     |                   | 122        | 188         | 18    | 16    | Shank            |
| 50  | 9563              | 121        | 183         | 18    | 16    | Shank            |
|     |                   | 120        | 160         | 10    | 9     | Threads          |
| 55  | 9564              | 122        | 163         | 10    | 9     | Threads          |
|     |                   | 130        | 165         | 8     | 8     | Threads          |
| 60  | 9565              | 119        | 179         | 17    | 14    | Threads          |
|     |                   | 122        | 177         | 15    | 12    | Threads          |
| 65  | 9571              | 126        | 188         | 15    | 13    | Threads          |
|     |                   | 121        | 178         | 15    | 11    | Threads          |
| 70  | 9572              | 129        | 191         | 17    | 13    | Threads          |
|     |                   | 122        | 180         | 14    | 11    | Threads          |
| 75  | 9573              | 141        | 208         | 25    | 29    | Shank            |
|     |                   | 141        | 215         | 24    | 27    | Shank            |
| 80  | 9574              | 143        | 216         | 24    | 31    | Shank            |
|     |                   | 141        | 214         | 25    | 32    | Shank            |
| 85  | 9575              | 149        | 223         | 23    | 28    | Shank            |
|     |                   | 156        | 220         | 24    | 31    | Shank            |
| 90  | 9573              | 149        | 200         | 12    | 9     | Threads          |
|     |                   | 153        | 201         | 11    | 9     | Threads          |
| 95  | 9574              | 162        | 209         | 11    | 9     | Threads          |
|     |                   | 151        | 206         | 14    | 13    | Threads          |
| 100 | 9575              | 157        | 218         | 22    | 27    | Shank            |
|     |                   | 160        | 224         | 23    | 31    | Shank            |
| 105 | 9573              | 158        | 221         | 16    | 13    | Threads          |
|     |                   | 148        | 214         | 16    | 12    | Threads          |
| 110 | 9574              | 165        | 224         | 24    | 32    | Shank            |

TABLE III

1,400° F. Tensile Results and Specimen Data

| CKB | Grain | YS, | UTS, | EL, | RA, | Failure |
|-----|-------|-----|------|-----|-----|---------|
|-----|-------|-----|------|-----|-----|---------|

TABLE V

| part Number | Size Range | K.s.i. | K.s.i. | %  | %  | Location |
|-------------|------------|--------|--------|----|----|----------|
| 9561        | Coarse     | 118    | 154    | 15 | 19 | Shank    |
|             |            | 117    | 151    | 22 | 34 | Shank    |
| 9562        | Coarse     | 120    | 160    | 19 | 21 | Shank    |
|             |            | 108    | 146    | 23 | 33 | Shank    |
| 9563        | Coarse     | 108    | 148    | 28 | 36 | Shank    |
|             |            | 118    | 154    | 26 | 30 | Shank    |
| 9564        | Coarse     | 114    | 147    | 18 | 31 | Shank    |
|             |            | 108    | 149    | 21 | 32 | Shank    |
| 9565        | Coarse     | 107    | 151    | 26 | 32 | Shank    |
|             |            | 116    | 154    | 21 | 26 | Shank    |
| 9571        | Fine       | 106    | 150    | 24 | 30 | Shank    |
|             |            | 107    | 150    | 23 | 25 | Shank    |
| 9572        | Fine       | 117    | 154    | 22 | 25 | Shank    |
|             |            | 122    | 152    | 16 | 16 | Shank    |
| 9573        | Fine       | 130    | 150    | 13 | 19 | Shank    |
|             |            | 130    | 157    | 11 | 15 | Shank    |
| 9574        | Fine       | 128    | 155    | 21 | 52 | Shank    |
|             |            | 128    | 149    | 23 | 55 | Shank    |
| 9575        | Fine       | 138    | 154    | 29 | 54 | Shank    |
|             |            | 136    | 150    | 34 | 58 | Shank    |
| 9576        | Fine       | 140    | 151    | 23 | 53 | Shank    |
|             |            | 159    | 169    | 30 | 52 | Shank    |
| 9577        | Fine       | 132    | 151    | 26 | 55 | Shank    |
|             |            | 131    | 147    | 23 | 59 | Shank    |
| 9578        | Fine       | 142    | 147    | 29 | 57 | Shank    |
|             |            | 132    | 151    | 10 | 14 | Threads  |
| 9579        | Fine       | 132    | 149    | 14 | 20 | Threads  |
|             |            | 137    | 154    | 31 | 57 | Shank    |

TABLE IV  
1400°F/85.0 ksi stress rupture results and specimen data

| CKB part number | Grain size range | Life, hr. | EL, percent | RA, percent | Failure location | Root Radius, Area Ratio, in. (Thousands) |         |         |         |
|-----------------|------------------|-----------|-------------|-------------|------------------|------------------------------------------|---------|---------|---------|
|                 |                  |           |             |             |                  | End One                                  | End Two | End One | End Two |
| 9561            | Coarse           | 50        | 8           | 8           | Threads          | 93                                       | 93      | 8       | 8       |
|                 |                  | 58        | 21          | 24          | Threads          | 93                                       | 93      | 8       | 8       |
|                 |                  | 43        | 9           | 12          | Shank            | 93                                       | 93      | 8       | 8       |
|                 |                  | 62        | 14          | 14          | Shank            | 93                                       | 93      | 8       | 8       |
| 9562            | Coarse           | 44        | 16          | 24          | Shank            | 93                                       | 93      | 8       | 8       |
|                 |                  | 50        | 19          | 25          | Shank            | 93                                       | 93      | 8       | 8       |
|                 |                  | 57        | 25          | 26          | Shank            | 93                                       | 93      | 8       | 8       |
|                 |                  | 53        | 23          | 29          | Shank            | 93                                       | 93      | 8       | 8       |
| 9563            | Coarse           | 40        | 16          | 27          | Shank            | 93                                       | 93      | 10      | 10      |
|                 |                  | 51        | 13          | 20          | Shank            | 93                                       | 92      | 10      | 10      |
|                 |                  | 52        | 18          | 19          | Shank            | 92                                       | 92      | 10      | 10      |
|                 |                  | 69        | 14          | 15          | Shank            | 92                                       | 92      | 10      | 10      |
| 9564            | Coarse           | 68        | 14          | 16          | Shank            | 93                                       | 93      | 10      | 10      |
|                 |                  | 48        | 19          | 25          | Shank            | 92                                       | 92      | 10      | 10      |
|                 |                  | 52        | 16          | 22          | Shank            | 93                                       | 93      | 10      | 10      |
|                 |                  | 61        | 17          | 18          | Shank            | 92                                       | 92      | 10      | 10      |
| 9565            | Coarse           | 54        | 15          | 20          | Shank            | 95                                       | 95      | 5       | 5       |
|                 |                  | 45        | 19          | 23          | Shank            | 95                                       | 95      | 5       | 6       |
|                 |                  | 62        | 15          | 17          | Shank            | 95                                       | 95      | 5       | 5       |
|                 |                  | 53        | 17          | 22          | Shank            | 95                                       | 95      | 5       | 6       |
| 9571            | Fine             | 13        | 3           | 3           | Threads          | 93                                       | 93      | 9       | 9       |
|                 |                  | 8         | 6           | 8           | Shank            | 92                                       | 92      | 8       | 8       |
|                 |                  | 15        | 1           | 1           | Threads          | 92                                       | 92      | 9       | 9       |
|                 |                  | 19        | 3           | 3           | Threads          | 92                                       | 92      | 9       | 9       |
| 9572            | Fine             | 29        | 41          | 64          | Shank            | 92                                       | 93      | 8       | 8       |
|                 |                  | 34        | 37          | 51          | Shank            | 92                                       | 92      | 8       | 8       |
|                 |                  | 30        | 49          | 53          | Shank            | 92                                       | 93      | 8       | 8       |
|                 |                  | 31        | 42          | 51          | Shank            | 92                                       | 92      | 8       | 8       |
| 9573            | Fine             | 22        | 35          | 55          | Shank            | 93                                       | 93      | 10      | 10      |
|                 |                  | 36        | 28          | 48          | Shank            | 92                                       | 92      | 10      | 10      |
|                 |                  | 39        | 34          | 52          | Shank            | 92                                       | 92      | 10      | 10      |
|                 |                  | 16        | 45          | 58          | Shank            | 93                                       | 93      | 10      | 10      |
| 9574            | Fine             | 20        | 37          | 51          | Shank            | 92                                       | 93      | 10      | 10      |
|                 |                  | 22        | 53          | 65          | Shank            | 92                                       | 93      | 10      | 10      |
|                 |                  | 30        | 45          | 60          | Shank            | 92                                       | 92      | 10      | 10      |
|                 |                  | 18        | 42          | 70          | Shank            | 92                                       | 92      | 10      | 10      |
| 9575            | Fine             | 63        | 29          | 44          | Shank            | 95                                       | 95      | 7       | 6       |
|                 |                  | 30        | 36          | 60          | Shank            | 96                                       | 95      | 7       | 6       |
|                 |                  | 44        | 35          | 48          | Shank            | 96                                       | 96      | 6       | 5       |
|                 |                  | 47        | 45          | 55          | Shank            | 96                                       | 96      | 5       | 6       |

1,300°F./65.0 K s.i./100 hr. Stress  
Relaxation Results and Specimen Data

| CKB part number | Grain size range | Location | Relaxation, % |
|-----------------|------------------|----------|---------------|
| 9561            | Coarse           | Shank    | 4             |
|                 |                  | Shank    | 6             |
| 9562            | Coarse           | Shank    | 10            |
|                 |                  | Shank    | 7             |
| 9563            | Coarse           | Shank    | 3             |
|                 |                  | Shank    | 2             |
| 9564            | Coarse           | Shank    | 3             |
|                 |                  | Shank    | 6             |
| 9565            | Coarse           | Shank    | 11            |
|                 |                  | Shank    | 9             |
| 9571            | Fine             | Shank    | 10            |
|                 |                  | Shank    | 8             |
| 9572            | Fine             | Shank    | 12            |
|                 |                  | Shank    | 14            |
| 9573            | Fine             | Shank    | 8             |
|                 |                  | Shank    | 13            |
| 9574            | Fine             | Shank    | 12            |
|                 |                  | Shank    | 18            |
| 9575            | Fine             | Shank    | 10            |
|                 |                  | Shank    | 16            |

TABLE VI

| Type of Test      | Test Conditions                | Influence of Grain Size* |        |
|-------------------|--------------------------------|--------------------------|--------|
|                   |                                | Fine                     | Coarse |
| Stress Relaxation | 1,300°F./65.0 K s.i. 100 hr. D | B                        |        |
| Stress Rupture    | 1,400°F./85.0 K s.i.           | D                        | B      |
| Life              |                                | B                        | D      |
| EL                |                                | B                        | D      |
| RA                |                                | B                        | D      |
| Tensile           | Room Temperature               | B                        | D      |
| YS                |                                | B                        | D      |
| UTS               |                                | B                        | D      |
| EL                |                                | B                        | D      |
| RA                |                                | B                        | D      |
| 65                | Tensile                        | 1,400°F.                 |        |
| YS                |                                | B                        | D      |
| UTS               |                                | N                        | N      |
| EL                |                                | B                        | D      |
| RA                |                                | B                        | D      |
| 70                |                                |                          |        |
|                   |                                |                          |        |

\*D = Detrimental Influence

B = Beneficial Influence

N = No Influence

The results confirm that both grain size and threading practice exert an influence on mechanical properties. The finer-grained specimens produced results equal or superior to the coarser-grained specimens in terms of all mechanical properties except stress rupture life and stress relaxation resistance. Unfortunately, the influence on grain size can be seen to exert contradictory effects in terms of the physical properties required of a threaded element. The choice of a grain size of ASTM 2-6 or more preferably ASTM 4-5 represents the best compromise for threaded elements, recognizing also the problems of precise grain size control in production processes.

Basically, the solution-roll-stabilize-age threading sequence improves the ability of the threads to resist stress relaxation and failure. It must, however, be considered in combination with the selection of the required grain size for optimum results. Clearly, the program has demonstrated that, as opposed to conventional processing techniques, the improved process described herein may be utilized to provide threaded elements which are not susceptible to thread failure.

While the invention has been described in connection with certain examples and preferred embodiments, these are illustrative only. It will be understood that the invention is not to be limited to the exact details described, for obvious modifications will occur to those skilled in the art.

We claim:

1. The process of fabricating threaded elements from the age-hardenable alloys which comprises:

forming the threads on solution heat treated, age-hardenable alloy stock having a grain size corresponding to about ASTM 2-6;

subjecting the threaded alloy to a stabilization heat treatment; and aging the alloy.

2. The process of fabricating threaded elements from the age-hardenable nickel-base alloy which comprises:

solution heat treating the alloy to establish a grain size substantially corresponding to ASTM 2-6;

rolling the threads; subjecting the threaded alloy to a stabilization heat treatment and precipitation heat treating the stabilized alloy.

3. The method of fabricating threaded elements for service up to about 1,200° F. which comprises:

providing suitable stock from an alloy consisting essentially of, by weight, about 18-21 percent chromium, 12-15 percent cobalt, 3.5-5 percent molybdenum, 2.75-3.25 percent titanium, 1.2-1.6 percent aluminum, about 0.07 percent carbon, about 0.005 percent boron, about 0.08 percent zirconium, balance nickel;

solution heat treating the alloy at 1,800°-1,900° F. for a minimum of about 2 hours and establishing a grain size corresponding to about ASTM 2-6;

rolling the threads in the stock after cooling; stabilization heat treating the alloy; and precipitation heat treating the alloy at about 1,400° F.

4. The process according to claim 3 wherein:

the stabilization heat treatment is conducted at a temperature of about 1,500° F.

5. The method of fabricating threaded elements for high-temperature service which comprises:

providing suitable stock from an alloy consisting essentially of, by weight, 14-16 percent chromium, 16-18 percent cobalt, 4.5-5.5 percent molybdenum, 3.35-3.65 percent titanium, 3.85-4.15 percent aluminum, about 0.06 percent carbon, about 0.03 percent boron, balance nickel;

solution heat treating the alloy at a temperature of at least 1,975° F. and establishing a grain size corresponding to about ASTM 2-6;

rolling the threads in the stock after cooling; stabilization heat treating the alloy; and precipitation heat treating the alloy at about 1,200° F.

6. The process according to claim 5 wherein: the stabilization heat treatment is conducted at a temperature of about 1,600° F.

\* \* \* \*

UNITED STATES PATENT OFFICE  
CERTIFICATE OF CORRECTION

Patent No. 3,615,906 Dated October 26, 1971

Inventor(s) Marvin C. Vanwanderham et al

It is certified that error appears in the above-identified patent and that said Letters Patent are hereby corrected as shown below:

Claim 3, column 6, line 13      1800° should read --1825°--  
Claim 4, column 6, line 21      1500° should read --1550°--

Signed and sealed this 28th day of March 1972.

(SEAL)

Attest:

EDWARD M.FLETCHER, JR.  
Attesting Officer

ROBERT GOTTSCHALK  
Commissioner of Patents